

# UNITED STATES PATENT OFFICE.

JOHN A. SHEPHERD, OF CLEVELAND, OHIO.

## WALL-COVERING.

SPECIFICATION forming part of Letters Patent No. 376,350, dated January 10, 1888.

Application filed January 13, 1887. Serial No. 224,279. (No specimens.)

*To all whom it may concern:*

Be it known that I, JOHN A. SHEPHERD, of Cleveland, in the county of Cuyahoga and State of Ohio, have invented certain Improvements 5 in Painted and Decorated Wall-Surfaces, of which the following is a specification.

The aim of my invention is to provide a painted and decorated wall-covering in sheet form, which shall be at once cheap and durable.

10 I first provide an adhesive or pasty compound, of such nature that when dry it will present a tough elastic body. I recommend, as best adapted for the purpose, a compound prepared as follows: In two gallons of hot water dissolve one pound of glue. To this solution add one pound of india-rubber dissolved in any ordinary or suitable manner, and after the rubber is thoroughly incorporated add one-half pound of corn-starch dis- 15 solved in hot water, and agitate the mass until all the ingredients are intimately united. I next provide a base sheet, of woven fabric, tough paper, or other analogous material, preferably, however, of cotton sheeting, and coat 20 the same thoroughly with the compound above described, and permit it to dry until it acquires what is technically known as a "tacky" condition. I then provide a surface-sheet of cheese-cloth, or similar fabric, saturate the 25 same with the compound, and, after spreading it upon the base-sheet, work it by hand or otherwise until it presents a wrinkled, waved, or other irregular surface, after which it is permitted to dry. The paste serves the 30 double purpose of uniting the two sheets and of stiffening the raised portions of the surface- sheet, and giving the same a sufficient body to keep it in form, combined with an elasticity or pliability such as to prevent it from crack- 35 ing or breaking. After the united sheets are dry I coat the surface-sheet with any appropriate paint, and ornament it by the application of gilt, bronze, mica, sand, flock, or other materials, according to taste. The resulting 40 product is a strong pliable body composed of two inseparable sheets or layers, one presenting a smooth surface adapted to be pasted or cemented to the wall, and the other present- 45 ing an irregular ornamental surface. Unlike

coverings made of rigid inflexible materials 50 and compounds, my covering may be rolled and bent without injury.

While I prefer to employ the adhesive stiffening compound above described, it is to be understood that any other suitable compound 55 of like character may be substituted therefor. It is to be further understood that the two sheets may be united by a cement or compound differing from that with which the surface- sheet is charged, if desired. 60

I am aware that it has been proposed to wrinkle paper by soaking the same in water, then squeezing and drying it, and that it has been proposed to paste the dried wrinkled sheet of paper upon another sheet, and when 65 the same was dried to harden the surface by shellacing or glue-sizing the same, and I lay no claim thereto.

It is to be noted, as a peculiarity of my product, that owing to the character of the fabric 70 from which it is made and the manner in which the fabric is treated the product has a pliable and elastic nature, so that it may be rolled for transportation, and that when in place it is free from liability to be cracked or 75 fractured.

Having thus described my invention, what I claim is—

1. A pliable wall covering consisting of a flat base-sheet of woven fabric and a wrinkled 80 surface-sheet of woven fabric, as cheese-cloth, the two cemented together and both charged or filled with sizing material, substantially as described.

2. In a wall-covering, a base sheet com- 85 bined with a wrinkled surface-sheet of woven material, as cheese-cloth, the two cemented together, and the surface sheet filled with a tough elastic material, substantially as set forth, whereby it is rendered pliable and pre- 90 vented from cracking.

In testimony whereof I hereunto set my hand, this 3d day of January, 1887, in the presence of two attesting witnesses.

JOHN A. SHEPHERD.

Witnesses:

SIDNEY P. HOLLINGSWORTH,  
WILLIAM H. SHIPLEY.